

Patented Sept. 18, 1951

2,568,180

# UNITED STATES PATENT OFFICE

2,568,180

## ALUMINUM BASE ALLOYS

Charles B. Willmore, North Aurora, Ill., assignor  
to William F. Jobbins, Incorporated, Aurora,  
Ill., a corporation of Illinois

No Drawing. Application April 12, 1949,  
Serial No. 87,110

5 Claims. (Cl. 75—141)

1

This invention relates to aluminum base alloys, and it has particular reference to the improvement in castability of aluminum base alloys, as measured by reduced surface shrinkage and less porosity in the casting. It also relates to the improvement in other physical properties of an aluminum base alloy containing zinc, copper and silicon as major alloying elements.

Aluminum base alloys of the type prescribed have been used in the manufacture of castings. They have not achieved wide commercial acceptance because they do not have desirable casting characteristics and their physical properties are not sufficiently superior to other commercial alloys having more desirable casting properties. One of the principal difficulties suffered by these alloys resides in the inability of securing an acceptable product by sand casting or by casting in permanent molds. By way of explanation, when the cast molten alloy cools down through the liquids range, the change from a liquid state to a solid state does not occur immediately. Instead, crystals or nuclei are formed which grow into a matrix having microscopic voids caused by the decrease in volume of the liquid as it assumes crystalline form. The voids that are formed are called pores when of small dimension and widely distributed, or pin holes, if the voids collect in certain areas.

These voids constitute low pressure areas and unless they are quickly filled, the casting surfaces may actually collapse to form depressed areas, characteristic of surface shrinkage, accompanied by undesirable crystal structure. Collapse to form surface shrinkage usually occurs in regions of relatively thick cross section. In the event that the matrix is sufficiently set to resist the effect of shrinkage forces, or in the event that gases originally dissolved in the metal fill the voids, the porosity defect remains as a permanent part of the casting. When either of these conditions prevail, a defective casting is produced which may be inadequate for the use for which it was intended.

Alloys of the type described are especially difficult to handle when casting about a core in permanent molds. Their inferior casting characteristics causes undesirable sticking of the core. This often leads to the destruction of the casting and excessive damage to the mold.

2

It is an object of this invention to provide an aluminum base alloy having improved castability when cast in sand or permanent molds.

Another object is to formulate for improvements in castability and other physical properties in an alloy composed chiefly of aluminum and containing silicon, copper and zinc as major alloying elements.

A further object is to provide an aluminum base alloy characterized by improved physical properties and improved castability when compared to alloys of corresponding composition heretofore produced.

Still another object is to provide a heat treatable aluminum base alloy containing silicon, zinc and copper as major alloying elements and characterized by improved castability and strength when fabricated by sand or permanent mold casting methods.

20 A still further object is to produce an aluminum base alloy having physical properties which may be improved by solution heat-treatment and which may be further improved by artificial aging.

25 This is a continuation-in-part of my co-pending application, Serial No. 87,109, filed on this same date and entitled "Aluminum Base Alloys" wherein description is made to the improvement in castability and physical properties

30 in an aluminum base alloy by the addition of chromium and/or manganese with or without titanium to an aluminum base alloy for casting in green sand or permanent molds. The additions of the minor alloying elements have particular merit when the aluminum base alloy is

35 constituted with copper, silicon and zinc as the major alloying elements present in amounts ranging from 2 to 4 percent copper, 2 to 8 percent zinc, 2 to 8 percent silicon and the sum of iron and nickel impurity is less than 0.75 percent.

40 I have discovered that physical properties of the desired character and improved castability may be secured by the addition with the elements employed in the parent application of a small amount of zirconium as an additional alloying element. By the further addition of zirconium, improvements are secured which cannot be achieved by a corresponding composition, devoid of zirconium or by increasing the ratio of elements chromium, manganese or titanium. Zir-

conium in amounts ranging from 0.05 to 0.30 percent is sufficient and best results are secured when zirconium in combination with chromium is added in an amount ranging from 0.10 to 0.25 percent.

Unlike chromium, zirconium offers some grain refining characteristics in either sand or chill casting whether chromium or titanium are present or not. Unlike titanium, however, zirconium is not detrimental to casting properties when chromium or manganese also is present. In chill or permanent mold casting, zirconium further improves castability with or without chromium, manganese and titanium.

These improved characteristics are shown by the following charts made from tests of aluminum base alloys containing impurities to the extent of 0.46 percent iron, 0.04 percent nickel and 0.15 percent manganese. Table I gives the physical properties developed by sand casting and Table II gives the physical properties developed by the particular alloy in permanent molds.

TABLE I

*Physical properties developed in sand casting*

|                                   |            |        |        |        |        |
|-----------------------------------|------------|--------|--------|--------|--------|
| Zinc.....                         | 5.4        | 5.4    | 5.4    | 5.4    | 5.4    |
| Copper.....                       | 3.0        | 3.0    | 3.0    | 3.0    | 3.0    |
| Silicon.....                      | 5.4        | 5.4    | 5.4    | 5.4    | 5.4    |
| Chromium.....                     | 0.25       | 0.25   | 0.25   | 0.25   | 0.25   |
| Zirconium.....                    | 0.19       | 0.19   | 0.19   | 0.19   | 0.19   |
| Titanium.....                     | 0.10       | 0.10   | 0.10   | 0.10   | 0.10   |
| Grain Size, diam. in mm.....      | 1.43       | 1.66   | 1.11   | 1.11   | 0.3    |
| Shrinkage.....                    | Very heavy | Slight | Medium | Slight | Medium |
| As Cast:                          |            |        |        |        |        |
| ultimate strength.....            | 25,500     | 26,500 | 26,300 | 26,900 | 26,200 |
| yield strength.....               | 13,000     | 13,000 | 14,800 | 15,600 | 14,900 |
| Heat Treated:                     |            |        |        |        |        |
| ultimate strength.....            | 32,900     | 33,700 | 32,400 | 31,500 | 36,800 |
| yield strength.....               | 16,900     | 16,300 | 16,300 | 16,700 | 17,200 |
| Heat Treated, Aged, ultimate..... | 46,200     | 46,900 | 44,700 | 47,900 | 44,900 |

TABLE II  
*Physical properties developed by permanent mold casting*

|                                   |             |        |        |        |        |
|-----------------------------------|-------------|--------|--------|--------|--------|
| Zinc.....                         | 5.4         | 5.4    | 5.4    | 5.4    | 5.4    |
| Copper.....                       | 3.0         | 3.0    | 3.0    | 3.0    | 3.0    |
| Silicon.....                      | 5.4         | 5.4    | 5.4    | 5.4    | 5.4    |
| Chromium.....                     | 0.25        | 0.25   | 0.25   | 0.25   | 0.25   |
| Zirconium.....                    | 0.19        | 0.19   | 0.19   | 0.19   | 0.19   |
| Titanium.....                     | 0.10        | 0.10   | 0.10   | 0.10   | 0.10   |
| Grain Size, diam. in mm.....      | 0.45        | 0.52   | 0.40   | 0.47   | 0.30   |
| Shrinkage.....                    | Very Medium | Slight | Slight | None   | None   |
| As Cast:                          |             |        |        |        |        |
| ultimate strength.....            | 30,000      | 30,900 | 29,800 | 30,100 | 31,800 |
| yield strength.....               | 13,450      | 12,400 | 15,300 | 15,700 | 16,000 |
| Heat Treated:                     |             |        |        |        |        |
| ultimate strength.....            | 36,500      | 38,400 | 40,900 | 41,200 | 39,600 |
| yield strength.....               | 16,400      | 16,900 | 17,000 | 16,800 | 16,700 |
| Heat Treated, aged, ultimate..... | 50,100      | 49,200 | 51,900 | 52,800 | 49,700 |

It will be apparent that the addition of zirconium alone to the base alloy gives certain reduction in grain size in both sand and permanent mold casting, a reduction which is far greater than that secured by the addition of chromium alone and less than a combination of chromium and zirconium but not less than that secured by the further addition of titanium. The addition of zirconium alone also gives improvement in castability, but the improvement is not as marked as that secured by the addition of zirconium in the present of chromium. Further, the addition of zirconium is more effective in most instances than an addition of chromium but the combination of zirconium and chromium with or without titanium gives best results in almost every case. While the physical data presented is for the system zirconium, chromium and titanium, it should be understood that corresponding results will be secured when manganese is used in whole

or in part for chromium, though ordinarily present in correspondingly larger proportion by weight.

As used in the tables, the term "heat treated" refers to solution heat treatment of the casting for 6 hours at 935 to 945° F. followed by quenching in hot water. Heat treatment time may be extended or shortened depending upon the weight of the casting, and heat treatment may be carried out at lower temperatures with a corresponding increase in time. The term "aged" refers to artificial ageing of the heat treated casting to precipitate out elements or compounds put into solid solution during heat treatment. Artificial ageing in the tested compositions was carried out by exposure of the heat treated casting to 305° to 315° F. for about three hours.

A very decided advantage is observed in the use of my new alloy in permanent mold casting. The alloy sets more rapidly in the mold with the consequent desirable advantage in that the molding cycle can be greatly shortened. For example, in one operation, a casting formed with my alloy composition can be removed after 1 to 1½ minutes in the mold, while a corresponding composition without zirconium and chromium or chromium and titanium requires a setting time of 1½ to 2 minutes. This enables the shortening of the time cycle by about 30 percent. Furthermore, the reduced shrinkage occasioned by the improved casting characteristics of the alloy permits casting in permanent molds without the difficulties heretofore occasioned upon casting about a core.

It will be apparent from the description that I have produced a new and improved aluminum base alloy containing zinc, copper and silicon, which alloy has greatly improved castability as measured by shrinkage and porosity and also has considerably better physical properties. The alloy corresponding to my invention is an alloy having desirable physical properties which may be improved by artificial ageing at relatively low temperatures.

It will be understood that changes may be made in the ratio of materials and compositions within the limitations prescribed and their method of treatment without departing from the spirit of the invention, especially as defined in the following claims.

What is claimed is:

1. An aluminum base alloy consisting essentially of 2 to 4 percent copper, 2 to 8 percent zinc, 2 to 8 percent silicon, 0.05 to 1.00 percent chromium, 0.05 to 0.30 percent zirconium, the balance being aluminum with less than 0.75 percent impurities made up of iron and nickel.

2. An aluminum base alloy consisting essentially of 2 to 4 percent copper, 2 to 8 percent zinc, 2 to 8 percent silicon, 0.05 to 1.0 percent chromium, 0.05 to 0.3 percent zirconium, 0.05 to 0.20 percent titanium, the balance being aluminum with less than 0.75 percent impurities made up of iron and nickel.

3. An aluminum base casting alloy consisting of from 2 to 4 percent copper, 4 to 8 percent zinc, 2 to 8 percent silicon, 0.10 to 0.45 percent chromium and 0.10 to 0.25 percent zirconium, the balance being aluminum with less than 0.75 percent impurities in the form of iron and nickel.

4. An aluminum base casting alloy consisting of from 2 to 4 percent copper, 4 to 8 percent zinc, 2 to 8 percent silicon, 0.10 to 0.45 percent chromium, 0.10 to 0.25 percent zirconium, and 0.05 to 0.15 percent titanium, the balance being alumi-

num with less than 0.75 percent impurities in the form of iron and nickel.

5. An aluminum base casting alloy consisting essentially of from 2 to 4 percent copper, 2 to 8 percent zinc, 2 to 8 percent silicon, an element selected from the group consisting of 0.05 to 1.00 percent chromium, 0.15 to 1.5 percent manganese and mixtures thereof, and 0.05 to 0.30 percent zirconium, the rest being aluminum with less than 0.75 percent impurities made up of iron and nickel.

CHARLES B. WILLMORE.

#### UNITED STATES PATENTS

| Number      | Name     | Date          |
|-------------|----------|---------------|
| 1,572,489   | Johnston | Feb. 9, 1926  |
| 2,043,855   | Keller   | June 9, 1936  |
| 5 2,098,081 | Bates    | Nov. 2, 1937  |
| 2,280,170   | Stroup   | Apr. 21, 1942 |
| 2,290,016   | Bonsack  | July 14, 1942 |

#### FOREIGN PATENTS

| Number     | Country       | Date          |
|------------|---------------|---------------|
| 10 576,230 | Great Britain | Mar. 25, 1946 |
| 864,251    | France        | Apr. 23, 1941 |

#### OTHER REFERENCES

15 "Manual of Aluminum Casting Alloys," published by the Aluminum Research Institute, Chicago, 1947, page 26.

#### REFERENCES CITED

The following references are of record in the 15 file of this patent: